

# United States Patent

[11] 3,615,511

[72] Inventor **Roger M. Cole**  
Rochester, N.Y.  
[21] Appl. No. **731,275**  
[22] Filed **May 22, 1968**  
[45] Patented **Oct. 26, 1971**  
[73] Assignee **Eastman Kodak Company**  
Rochester, N.Y.

3,396,017 8/1968 Bacon et al. .... 96/63 X  
3,418,124 12/1968 Hunt ..... 96/61

## OTHER REFERENCES

Mees—James: The Theory of the Photographic Process, 3rd Edition, page 122, 1966.

Primary Examiner—Norman G. Torchin

Assistant Examiner—Won H. Louie, Jr.

Attorneys—W. H. J. Kline, G. E. Battist and B. D. Wiese

[54] **SURFACE DEVELOPER WITH HETEROCLIC MERCAPTAN FOR USE ON INTERNAL IMAGE EMULSION**  
13 Claims, No Drawings

[52] U.S. Cl. .... **96/61**,  
96/108, 96/63, 96/66.5  
[51] Int. Cl. .... **G03c 5/38**  
[50] Field of Search ..... 96/108, 61,  
63, 66.5, 66

[56] **References Cited**  
UNITED STATES PATENTS

3,335,009 8/1967 Rasch et al. .... 96/61  
3,241,971 3/1966 Kitze ..... 96/108 X

**ABSTRACT:** Processes and compositions for developing or stabilizing image records in photographic, internal image, silver halide compositions. In one aspect, the developing or stabilizing compositions of this invention contain low concentrations of a silver complexing agent. In another aspect, photographic compositions are stabilized or developed with a process comprising a bleach bath followed by a surface type developer. In a preferred embodiment direct-print materials containing either photodeveloped images or nonphotodeveloped latent images can be processed to provide permanent image records.

SURFACE DEVELOPER WITH HETEROCLIC  
MERCAPTAN FOR USE ON INTERNAL IMAGE  
EMULSION

This invention relates to processes and compositions for developing or stabilizing image records in photographic materials. In one aspect this invention relates to novel processes for developing or stabilizing image records in direct-print, photographic materials. In another aspect, this invention relates to novel processes comprising bleaching and then developing or stabilizing image records in direct-print material. In still another aspect, this invention relates to a means by which both latent images and photodeveloped images can be made into stable, permanent image records.

It is often desirable to permanize (i.e., to make permanent archival quality records) the image records in printout or direct-print compositions. Many printout and direct-print compositions produce high background density when the image records are subjected to conventional developers. The increase in background fog is especially a problem when photodeveloped direct-print records are stabilized or developed in conventional developers; in this instance photolytic silver is generally formed in both the image and background areas of the record. Moreover, single developing or stabilizing compositions known in the present art generally can not be successfully used to provide good stable image properties in both nonphotodeveloped and photodeveloped direct-print compositions. Therefore, improved means to obtain good stabilized records in printout or direct-print emulsions would be desirable.

It is an object of this invention to provide new means for stabilizing or developing internal image silver halide photographic compositions.

It is another object of this invention to provide new means for stabilizing or developing direct-print and printout photographic compositions.

It is another object of this invention to provide a means for producing a uniform image in a direct-print record which has been photodeveloped over only a portion of the record area.

It is another object of this invention to provide novel compositions for developing or stabilizing photographic compositions.

These and other objects of the invention have been accomplished by processing internal image silver halide materials in a surface developer containing low concentrations of a selective silver complexing agent and a silver halide developing agent. The surface developer is substantially free of strong silver halide solvents such as thiocyanates, hypo, etc. It is quite unexpected that low concentration of the selective silver complexing agents would provide improved development properties in this system since higher concentrations of the same compounds do not exhibit the same improvements in the development characteristics of the system. It is even more unexpected that this system can be used to permanize good images in both nonphotodeveloped and photodeveloped direct-print compositions.

In one embodiment, direct-print compositions which have been imagewise exposed are processed in a surface developer containing selective silver complexing agent, fixed and washed.

In another embodiment, direct-print records which have been imagewise exposed are photodeveloped to a discernible image and then processed in a surface developer containing a selective silver complexing agent, fixed and washed.

In another embodiment, direct-print compositions which have been imagewise exposed are bleached and then processed in a surface developer containing a selective silver complexing agent, fixed and washed.

In still another embodiment, direct-print compositions which have been imagewise exposed are photodeveloped, bleached, processed in a surface developer containing a selective silver complexing agent, fixed and washed.

The selective silver complexing agents of this invention contain two characteristic groups which provide the unique pro-

perties in the surface developers. The silver complexing agents contain at least one group which is capable of forming a normal covalent bond with silver. Typical complexing agents contain groups capable of forming the covalent bonds such as



and the like. The preferred complexing agents contain imide groups



mercaptan groups ( $-\text{SH}$ ) and the like or tautomers thereof. The complexing agents also contain at least one secondary bonding group which does not generally form a covalent bond with silver under the conditions generally encountered in photographic emulsions and photographic developing solutions. Bonds of this type are sometimes referred to as  $\pi$  bonds in the atomic configuration of the ion complex formation. Typical groups in the silver complexing agents of this invention which can be classified as secondary bonding groups are (1)



or carbon-carbon double bond groups; these groups can occur for example as part of a heterocyclic ring system as in 2-mercaptoimidazole or in an alkyl side chain as in 1-allyl-2-thiourea, (2) aromatic substituents; typical compounds of this type are benzo or phenyl derivatives, (3) donor atoms containing 2 nonbonding electron pairs; typical preferred groups of this type are



$-\text{S}-\text{S}-$  and the like.

The silver complexing agents of this invention can be additionally characterized as compounds which are soluble in water at 70°F. in concentration of at least  $10^{15}$  and preferably  $10^{12}$  moles per liter and wherein said compounds are capable of forming a silver ion complex in a ratio of at least 10 silver ion to 10 complexing agent on a molar basis in the presence of an equal molar or excess of silver ion as measured by potentiometric titration.

The silver complexing agents of this invention are incorporated in the developing solutions in lower concentrations than normally used for antifogging purposes. In embodiments wherein the developing solution is used directly after imagewise exposure or photodevelopment it is critical to maintain the concentration level of the silver complexing agent at levels below  $2 \times 10^{13}$  moles per liter of solution and preferably below  $1.5 \times 10^{13}$  moles per liter of developing solution. The concentrations of the silver complexing agent for this embodiment are maintained between about  $10^{15}$  moles to about  $2 \times 10^{13}$  moles per liter about  $1 \times 10^{14}$  moles to about  $1.5 \times 10^{13}$  moles per liter. In embodiments where a bleach bath is used prior to the developing bath the concentration of the silver complexing agent can be generally from about  $10^{15}$  moles to about  $4 \times 10^{13}$  moles and preferably from about  $10^{14}$  moles to not more than  $2.5 \times 10^{13}$  moles of solution. If the concentrations of the silver complexing agent exceed the above concentrations, the density of the developed image is greatly reduced.

In a preferred embodiment of this invention, direct-print compositions are stabilized or developed by contacting said compositions with a bleach bath and then contacting said compositions with the developing solutions containing the silver complexing agents. However, the bleach bath will also provide some improvements in image properties in direct-print emulsions when said bleach bath is followed with other developing solutions.

Typical compounds which can be characterized by the above tests and are effective in the developing baths of this in-

vention are 2-mercaptopthiazole, 2-mercaptopbenzothiazole, 2-mercaptop-6-nitrobenzothiazole, 4-carboxymethyl-4-thiazoline-2-thione, thiazolidine-2-thione, imidazole, 2-benzimidazolethiol, 5-amino-2-benzimidazolethiol, 2-mercaptopimidazole, 1-methyl-2-mercaptopimidazole, 2-mercaptopypyrimidine, dithiourazole, o-aminobenzeneethiol, o-mercaptopbenzoic acid, 1-phenyl-2-mercaptopetrazole, 1-phenyl-2-thiourea, 5-nitrobenzimidazolethiol, 6-amino-2-mercaptopbenzothiazole, 2-benzoxazolethiol, 5-methyl-2-oxazolidinethione, 4-aminophenyldisulfide and 1-allyl-2-thiourea.

In some instances the silver halide emulsions which can be processed according to this invention contain small amounts of compounds which have the characteristics of the above silver complexing agents. This is often the case with direct-print materials wherein halogen acceptors of this type are used in the compositions. However, the halogen acceptor concentration which is utilized to provide optimum image characteristics in a direct-print emulsion upon photodevelopment is generally too low to successfully provide the necessary image properties in a surface developer when permanizing the image record. The image record in direct-print emulsions containing these compounds as halogen acceptors are greatly improved by the use of the indicated concentrations of the silver complexing agent in the surface developer baths according to this invention.

The bleach baths which can be used in certain preferred embodiments of this invention include baths containing oxidizing agents such as, for example, those disclosed in *The Journal of Photographic Science*, Vol. 9, 1961, pp. 217-222. Generally the oxidizing agent concentrations of baths used in this invention is from about one gram/liter to about 100 gram/liter and preferably from about 5 grams to about 50 grams per liter.

The developing bath comprises any of the conventional developing agents used for surfaces development of photographic records. Typical developing agents include hydroquinone, ascorbic acid, 1-hydroxy-2-methylaminobenzene, catechol, pyrogallol, 1-phenyl-3-pyrazolidone, para-hydroxyphenyl-aminoacetic acid, t-butyl-hydroquinone, 4-methyl-4-hydroxymethyl-1-phenyl-3-pyrazolidone and the like.

It is understood that the developing baths of this invention are substantially free of strong silver halide solvents or fixing agents such as water soluble thiocyanates and thiosulfates such as potassium thiocyanate and sodium thiosulfate. The presence of such strong silver halide solvents destroys the equilibrium balance necessary to obtain good results by the process of this invention.

The silver halide compositions which can be stabilized or developed according to this invention are those which are internally sensitive to electromagnetic radiation, i.e., light, X-rays, electrons, etc. Suitable silver halides include internally sensitive silver bromide, silver bromoiodide, silver chlorobromide, silver chlorobromoiodide, and the like. The preferred emulsions are those wherein the silver halide is predominately silver bromide. In a typical embodiment preferred emulsions according to this invention have higher internal sensitivity than surface sensitivity. Typical suitable emulsions are disclosed in Davey et al., U.S. Pat. No. 2,592,250 issued Apr. 8, 1952; U.S. Pat. No. 3,206,316; Porter et al., U.S. Pat. No. 3,206,313 Glafkides, *Photographic Chemistry*, Vol. 1, pp. 31-32, Fountain Press, London; McBride, U.S. Pat. No. 3,271,157 issued Sept. 6, 1966, McBride U.S. Pat. No. 3,287,137 issued Nov. 22, 1966, and Hunt, *Photographic Science and Engineering*, Vol. 5, No. 2, Mar.-Apr., 1961, pp. 104-108.

The so-called "internal image" emulsions can be used in the invention, such having silver halide grains wherein a predominant amount of the sensitivity is internal to the grains. Such internal image emulsions are those which, when measured according to normal photographic techniques by coating a test portion of the emulsion on a transparent support, exposing to

a light intensity scale having a fixed time between  $1 \times 10^{16}$  and 10 second, bleaching 5 minutes in a 0.3 percent potassium ferricyanide solution at 65° F., and then developing in Developer Z below (an "internal-type" developer), have a sensitivity measured at a density of 0.1 above fog, greater than the sensitivity of an identical test portion which has been exposed in the same way and developed for 6 minutes at 68° F. in Developer X below (a "surface-type" developer).

#### DEVELOPER X

|    |                                |         |
|----|--------------------------------|---------|
| 10 | N-Methyl-p-aminophenol sulfate | 0.31 g. |
|    | Sodium sulfite, desiccated     | 39.6 g. |
|    | Hydroquinone                   | 6.0 g.  |
|    | Sodium carbonate, desiccated   | 18.7 g. |
|    | Potassium bromide              | 0.86 g. |
|    | Citric acid                    | 0.68 g. |
|    | Potassium metabisulfite        | 1.5 g.  |
|    | Water to make 1 liter          |         |

#### DEVELOPER Z

|    |                                |         |
|----|--------------------------------|---------|
| 20 | N-Methyl-p-aminophenol sulfate | 2.0 g.  |
|    | Sodium sulfite, desiccated     | 90.0 g. |
|    | Hydroquinone                   | 8.0 g.  |
|    | Sodium carbonate, monohydrate  | 52.5 g. |
|    | Potassium bromide              | 5.0 g.  |
|    | Sodium thiosulfate             | 10.0 g. |
|    | Water to make 1 liter          |         |

The direct-print emulsions which can be stabilized in accordance with this invention generally contain halogen acceptors, for example, nitrogen containing halogen acceptors such as those disclosed in McBride, U.S. Pat. No. 3,287,137 and McBride, U.S. Pat. No. 3,271,157.

In certain preferred emulsions to be stabilized or developed by the methods of this invention, it is desirable to add water-soluble halides to the silver halide emulsion after its precipitation but before it is coated. More generally, about 1 to about 50 mole percent, and preferably about 1 to about 10 mole percent of water soluble halide based on the silver halide in the emulsion is used.

The stabilizing or developing baths of this invention can also be used to treat other silver halide systems, such as developing out system, etc., if desired to maintain or improve image properties in said systems.

Various colloids can be used as vehicles or binding agents in preparing the silver halide emulsions of this invention. Satisfactory colloids which can be used for this purpose include any of the hydrophilic colloids generally employed in the photographic field including, for example, gelatin, colloidal albumin, polysaccharides, cellulose derivatives, synthetic resins such as polyvinyl compounds, including polyvinyl alcohol derivatives, acrylamide polymers and the like. In addition to the above hydrophilic colloids, the vehicle or binding agent can also contain hydrophobic colloids such as dispersed polymerized vinyl compounds, particularly those which increase the dimensional stability of photographic materials. Suitable compounds of this type include water-soluble polymers of alkyl acrylates or methacrylates, acrylic acid, sulfoalkyl acrylates or methacrylates, and the like.

The above-described emulsions of the invention can be coated on a wide variety of supports in accordance with usual practice. Typical supports for photographic elements of the invention include glass, metal, paper, polyolefin-coated paper, cellulose nitrate film, cellulose acetate film, polystyrene film, polyester films such as polyethylene terephthalate film, heat resistant polymeric films such as high temperature polyester, polyimide, polycarbonate films, and the like.

The essential ingredients of the stabilizing compositions according to the invention, namely the developing agents, the selective silver complexing agent and in some embodiments,

the bleach, can be prepackaged in a kit, diluted, concentrated, or in powder form and can be either mixed together or packaged individually for use in the systems of this invention. The respective compositions are generally prepackaged individually and can be readily added to aqueous alkaline solution or water to form the necessary baths. Therefore it is understood that kits prepared for making stabilizing compositions comprising the essential ingredients of this invention are contemplated to be within the scope of this invention.

The invention can be further illustrated by the following examples.

#### EXAMPLE 1

Strips of a direct-print silver halide emulsion prepared according to example 1d of McBride U.S. Pat. No. 3,287,136 are imagewise exposed to a step tablet on a sensitometer by exposing for  $10^{14}$  second to a high intensity Xenon light. The respective samples are subsequently photodeveloped by exposing to 250 foot-candles of daylight fluorescent illumination for 30 seconds to produce a negative image with about 0.4 density discrimination.

One of the samples is processed in Developer A., described below, for 60 seconds, then stopped in acetic acid for 10 seconds, fixed for 2 minutes in sodium thiosulfate solution and washed for 5 minutes in running water.

A second sample is processed by the above procedure wherein Developer A additionally contains 0.1 g./l. of 1-phenyl-5-mercaptopterazole.

#### EXAMPLE 2

Samples of direct-print silver halide emulsions prepared according to example 11 of Kitz, Belgian Pat. No. 689,515 issued Jan. 13, 1967, are imagewise exposed to a step tablet on a sensitometer by exposing for  $10^{14}$  second to a high intensity Xenon light. The respective samples are subsequently photodeveloped by exposing to 50 foot-candles of fluorescent illumination for 2 minutes. The density of the image area and the background area are shown in table I.

One of the photodeveloped samples is processed as a control sample in Developer B for 60 seconds, then stopped for 10 seconds, fixed for 5 minutes and washed for 5 minutes. The image record densities obtained for this process are shown in table I.

#### DEVELOPER B

|                      |           |
|----------------------|-----------|
| Methyl-p-aminophenol | 4.5 g./l. |
| Hydroquinone         | 9 g./l.   |
| Sodium sulfite       | 50        |
| Sodium carbonate     | 80        |
| Potassium bromide    | 2         |

Several additional nonphotodeveloped and photodeveloped samples are processes in Developer B containing the concentrations of selective silver complexing agents indicated in table I. The densities of the image area obtained upon development are recorded in table I.

TABLE I

| Developer   | Silver complexing agent          | Concen-<br>tration,<br>g./l. | Non-phdvlpd<br>density |       | Phdvlpd<br>density |       |
|-------------|----------------------------------|------------------------------|------------------------|-------|--------------------|-------|
|             |                                  |                              | Bkgrnd                 | Image | Bkgrnd             | Image |
| None        | None                             |                              |                        |       | 0.38               | 0.68  |
| Developer B | None                             |                              | 0.14                   | 1.24  | 0.56               | 0.49  |
| Do          | 2-mercaptopimidazole             | 0.1                          | 0.12                   | 1.18  | 0.52               | 0.85  |
| Do          | do                               | 0.01                         |                        |       |                    |       |
| Do          | 2-thiouracil                     | 0.1                          | 0.14                   | 1.21  | 0.64               | 0.91  |
| Do          | do                               | 0.01                         | 0.15                   | 1.21  | 0.58               | 0.64  |
| Do          | 2,5-dimercapto-1,2,4-thiadiazole | 0.1                          | 0.20                   | 1.23  | 0.62               | 0.82  |
| Do          | do                               | 0.01                         | 0.18                   | 1.22  | 0.49               | 0.53  |
| Do          | Dithiourazole                    | 0.1                          | 0.16                   | 1.24  | 0.60               | 0.84  |
| Do          | 2,5-dithiobiurea                 | 0.01                         | 0.19                   | 1.22  | 0.48               | 0.49  |
| Do          | 2,5-dithiobiurea                 | 0.1                          | 0.16                   | 1.22  | 0.62               | 0.80  |
| Do          | 2-thioorotic acid                | 0.01                         | 0.16                   | 1.24  | 0.52               | 0.53  |
| Do          | 2-thioorotic acid                | 0.1                          | 0.16                   | 1.22  | 0.55               | 0.73  |
| Do          | 2,6-dimercapto-purine            | 0.1                          | 0.19                   | 1.24  | 0.60               | 0.83  |
|             |                                  | 0.01                         | 0.18                   | 1.24  | 0.55               | 0.50  |

#### DEVELOPER A

|                                  |         |
|----------------------------------|---------|
| Water                            | 800 ml. |
| N-methyl-p-aminophenol           | 6 g.    |
| Sodium isocorboxate              | 40 g.   |
| Potassium bromide                | 1 g.    |
| Kodalk                           | 40 g.   |
| 4-methyl-1-phenyl-3-pyrosolidone | 1 g.    |
| Water to make 1 liter            |         |

The above data demonstrates that good image densities can be obtained with either photodeveloped or nonphotodeveloped direct-print samples which are processed with surface developers containing low concentrations of silver complexing agents.

When the 2-mercaptopimidazole as used in the developer is replaced with imidazole, 1-allyl-2-thiourea or o-mercaptopbenzoic acid similar improvements in photographic properties are obtained.

| Sample                                     | Background<br>Density | Image<br>Density | 60 |
|--------------------------------------------|-----------------------|------------------|----|
| Developer A                                | 0.48                  | 0.46             |    |
| Developer A + 1-phenyl-5-mercaptopterazole | 0.67                  | 1.01             | 65 |

The addition of 1-phenyl-5-mercaptopterazole to the developer prevented the image reversal and promoted development of the high intensity exposure areas producing a negative image corresponding to the photodeveloped image which is normally obtained in a direct-print material.

Similar results are obtained when less than 150mg. of 2-mercaptopimidazole, dithiourazole, 1-allyl-2-thiourea, 4-carboxymethyl-4-thiazoline-2-thione and o-mercaptopbenzoic acid are utilized in the developer.

#### EXAMPLE 3

A bleach bath is preferably used when processing a direct-print emulsion prior to processing in the developer containing selective silver complexing agents.

A direct-print silver halide emulsion prepared according to example 1d of McBride U.S. Pat. No. 3,287,136 is imagewise exposed on a sensitometer using a  $10^{14}$  second flash with a high intensity Xenon lamp. The sample is then photodeveloped by exposing it to 250 foot-candles of daylight fluorescent illumination for 2 minutes.

A control sample is processed in Developer A for 2 minutes, fixed for 5 minutes and washed in running water. A second sample of the above emulsion is processed in Developer C according to the same processing procedure.

## DEVELOPER C

|                                |         |
|--------------------------------|---------|
| Water                          | 800 ml. |
| N-methyl-para-aminophenol      | 6 g.    |
| Sodium isoascorbate            | 40 g.   |
| Potassium bromide              | 1 g.    |
| Kodak Balanced Alkali          | 40 g.   |
| 4-methyl-phenyl-3-pyrazolidone | 1 g.    |
| 1-phenyl-5-mercaptopurine      | 0.1 g.  |
| water to make 1 liter          |         |
| pH=10.0                        |         |

Additional samples prepared by the above procedure are treated with an oxidizing bath, Bleach A, for 2 minutes, then processed in a manner similar to the control sample.

## BLEACH A

|                       |         |
|-----------------------|---------|
| Potassium dichromate  | 7.5 g.  |
| Sulfuric acid (conc.) | 5.0 ml. |
| Water to              | 1 liter |

The combination of the bleach bath and the developer containing the selective silver complexing agents produces lower minimum density with better image discrimination than the developer containing the selective silver complexing agents alone or the bleach followed by the conventional surface developer.

TABLE II

| Bleach | Dev. | Reflection Densities |       |
|--------|------|----------------------|-------|
|        |      | Background           | Image |
| None   | A    | 0.55                 | 0.48  |
| None   | C    | 0.51                 | 0.88  |
| A      | A    | 0.47                 | 0.30  |
| A      | C    | 0.43                 | 0.87  |

Example 4

Samples of direct-print silver halide emulsions prepared according to example 4 of Karlson, Belgian Pat. No. 705,036 issued Nov. 14, 1967 (which contains a urazole halogen acceptor) are imagewise exposed to a step tablet on a sensitometer by exposing for  $10^{14}$  second with a high intensity Xenon light. The respective samples are subsequently photodeveloped by exposing to 50 foot-candles of daylight fluorescent illumination for 5 minutes. One of the photodeveloped samples is processed as a control sample in Developer D for 1 minute, fixed for 30 seconds and washed in running water. Another sample is processed for the same duration in Developer E.

## DEVELOPER D

|                           |         |
|---------------------------|---------|
| N-methyl-para-aminophenol | 4.5 g.  |
| Sodium sulfite            | 50.0 g. |
| Hydroquinone              | 9.0 g.  |
| Sodium carbonate          | 80.0 g. |
| Potassium bromide         | 2.0 g.  |
| Water to                  | 1 liter |

## DEVELOPER E

|                           |        |
|---------------------------|--------|
| N-methyl-para-aminophenol | 4.5 g. |
|---------------------------|--------|

|                   |         |
|-------------------|---------|
| Sodium sulfite    | 50.0 g. |
| Hydroquinone      | 9.0 g.  |
| Sodium carbonate  | 80.0 g. |
| Potassium bromide | 2.0 g.  |
| 2-mercaptopurine  | 0.1 g.  |
| Water to          | 1 liter |

A photodeveloped sample is prepared as above and then bathed in an oxidizing bath (Bleach B) for 1 minute, then processed in an identical manner as the control. The density data obtained is shown in Table III.

## BLEACH B

|                       |         |
|-----------------------|---------|
| Potassium dichromate  | 20 g.   |
| Sulfuric acid (conc.) | 4 ml.   |
| Water to              | 1 liter |

TABLE III

| Bleach | Dev. | Transmission Densities |       |
|--------|------|------------------------|-------|
|        |      | Background             | Image |
| None   | D    | 0.72                   | 1.12  |
| None   | E    | 0.65                   | 1.22  |
| B      | D    | 0.12                   | 0.22  |
| B      | E    | 0.25                   | 0.66  |

The normal surface developer produced a negative image with high background density; while the bleach process followed by the developer containing the selective silver complexing agent greatly reduced the background and maintained equivalent image discrimination. The resulting image produced by the bleach process followed by the developer containing the selective silver complexing agent provides a record which is much more discernible to the eye as the image density is on a percentage basis much darker than the background density. Similar results are obtained when 1-allyl-2-thiourea, imidazole, dithiourazole, and 1-phenyl-2-thiourea are utilized in Developer E in place of the 2-mercaptopurine.

## EXAMPLE 5

A control direct-print emulsion is prepared according to example 1a of Kitze, Belgian Pat. No. 689,515, issued Jan. 13, 1967. Another sample (sample A) of a similar emulsion is prepared by the same procedure with the addition of 15 g./mole of silver of 2-mercaptopurine incorporated in the emulsion coating. Samples of the respective coatings are exposed for  $10^{14}$  second to a high intensity Xenon lamp through a 0 to 3.0 neutral density step tablet on a sensitometer. The images are then photodeveloped with 245 foot-candles of daylight fluorescent light for 30 seconds. The respective photodeveloped samples are solution processed at 70° F. in the following solutions as indicated in table IV.

| 60 | Bleach A              | 30 seconds |
|----|-----------------------|------------|
|    | Potassium dichromate  | 20 g./l.   |
|    | Sulfuric Acid (conc.) | 4 g./l.    |

| 65 | DEVELOPER F               | 60 seconds |
|----|---------------------------|------------|
|    | N-methyl-para-aminophenol | 3.1 g.     |
|    | Hydroquinone              | 12.0 g.    |
|    | Sodium sulfite            | 45.0 g.    |
|    | Sodium carbonate          | 80.0 g.    |
|    | Potassium bromide         | 1.9 g.     |
|    | Water to                  | 1 liter    |

|                    |          |            |
|--------------------|----------|------------|
| Sodium thiosulfate | 140.0 g. | 60 seconds |
| Sodium sulfite     | 15.0 g.  |            |
| Water to           | 1 liter  |            |

Wash Running Water

2 minutes

Additional samples are processed by the above procedure except Developer G was substituted for Developer F on the procedure. Developer G is identical in all respects to Developer F with the addition of 0.075 g./l. of 2-mercaptopimidazole.

The densities obtained in the respective photographic samples are reported in table IV below.

TABLE IV

| Sample  | Developer F |       |      | Developer G |       |      |
|---------|-------------|-------|------|-------------|-------|------|
|         | Back-ground | Image | ΔD   | Back-ground | Image | ΔD   |
| Control | 0.28        | 0.26  | 0.02 | 0.30        | 0.57  | 0.27 |
| Control |             |       |      |             |       |      |
| A       | 0.34        | 0.64  | 0.30 | 0.38        | 0.76  | 0.38 |
| A       |             |       |      |             |       |      |

The selective silver complexing agent utilized in the emulsion shows an improvement in discrimination over the process without agent present. Moreover, the addition of the selective silver complexing agent in the developer in addition to the use of the same or a similar compound in the emulsion coating shows an additional improvement in the image discrimination obtained after processing.

The invention has been described in considerable detail with reference to preferred embodiments thereof, but it will be understood that variations and modifications can be effected within the spirit and scope of the invention as described hereinabove and in the appended claims.

I claim:

1. A process for developing and stabilizing image records in an internal image silver halide compositions which has been imagewise exposed comprising contacting said silver halide composition with a surface developing solution, said solution comprising a developing agent and from  $10^{15}$  moles/liter to about  $2 \times 10^{13}$  moles/liter of a silver complexing agent, said complexing agent containing at least one group capable of forming covalent bonds with silver said group selected from mercaptan groups, imide groups, or tautomers thereof and at least one secondary bonding group capable of forming pi-bonds, said secondary bonding group consisting of



groups.

2. A process according to claim 1 wherein said groups capable of forming covalent bonds with silver consist of mercaptan groups.

3. A process according to claim 2 wherein said silver complexing agent is 2-mercaptopimidazole.

4. A process according to claim 1 wherein said silver complexing agent is selected from the group consisting of 2-mercaptopthiazole, 2-mercaptopbenzothiazole, 2-mercaptop-6-nitrobenzothiazole, 4-carboxymethyl-4-thiazoline-2-thione, thiadiazoline-2-thione, imidazole, 2-benzimidazolethiol, 5-amino-2-benzimidazolethiol, 2-mercaptopimidazole, 1-methyl-2-mercaptopimidazole, 2-mercaptopurimidine, dithiourazole, o-aminobenzenethiol, o-mercaptopbenzoic acid, 1-phenyl-2-mercaptoptetrazole, 1-phenyl-2-thiourea, 5-nitrobenzimidazolethiol, 6-amino-2-mercaptopbenzothiazole, 2-benzoxazolethiol, 5-methyl-2-oxazolinethione, 4-aminophenyl-disulfide and 1-allyl-2-thiourea.

5. A process according to claim 4 wherein said silver complexing agent is selected for the group consisting of 1-allyl-2-thiourea, 2-mercaptopimidazole, dithiourazole, and 1-phenyl-5-mercaptoptetrazole. 3

6. A process according to claim 4 wherein said silver complexing agent is 2-mercaptopimidazole, in a concentration of from  $1 \times 10^{14}$  to about  $1.5 \times 10^{13}$  moles/liter.

7. A process for stabilizing image records in light developable internal image silver halide compositions which have been imagewise exposed and photodeveloped to produce a visible image therein, said process comprising (1) contacting said silver halide composition with a silver halide bleaching solution, and then (2) contacting said silver halide with a surface developing solution comprising a developing agent and from about  $10^{15}$  to about  $4 \times 10^{13}$  moles/liter of a silver complexing agent comprising at least one group capable of forming covalent bonds with silver, said groups selected from mercaptan groups, imide groups, or tautomers thereof and at least one secondary bonding group capable of forming pi-bonds, said secondary bonding group consisting of



groups.

8. A process according to claim 7 wherein said silver complexing agent is selected from a group consisting of 2-mercaptopthiazole, 2-mercaptopbenzothiazole, 2-mercaptop-6-nitrobenzothiazole, 4-carboxymethyl-4-thiazoline-2-thione, thiadiazoline-2-thione, imidazole, 2-benzimidazolethiol, 5-amino-2-benzimidazolethiol, 2-mercaptopimidazole, 1-methyl-2-mercaptopimidazole, 2-mercaptopurimidine, dithiourazole, o-aminobenzenethiol, o-mercaptopbenzoic acid, 1-phenyl-2-mercaptoptetrazole, 1-phenyl-2-thiourea, 5-nitrobenzimidazolethiol, 6-amino-2-mercaptopbenzothiazole, 2-benzoxazolethiol, 5-methyl-2-oxazolinethione, 4-aminophenyl-disulfide and 1-allyl-2-thiourea.

9. A process according to claim 7 wherein said silver complexing agent is selected from the group consisting of 1-allyl-2-thiourea, 2-mercaptopimidazole, dithiourazole, and 1-phenyl-5-mercaptoptetrazole.

10. A process according to claim 7 wherein said bleaching solution comprises potassium dichromate, and said silver complexing agent comprises 2-mercaptopimidazole.

11. A process according to claim 7 wherein said groups capable of forming covalent bonds with silver consists of mercaptan groups.

12. A process according to claim 7 wherein said silver complexing agent is 2-mercaptopimidazole.

13. A process according to claim 7 wherein said silver complexing agent is compound which is soluble in water in a concentration of at least  $10^{15}$  moles/liter at 70° F. and wherein said compound is capable of forming a silver complex having a ratio of at least 1 silver ion to 1 silver complexing agent in a molar basis in the presence of excess silver ions as measured by potentiometric titration.

\* \* \* \* \*

UNITED STATES PATENT OFFICE  
CERTIFICATE OF CORRECTIONPatent No. 3,615,511Dated October 26, 1971Inventor(s) Roger M. Cole

It is certified that error appears in the above-identified patent and that said Letters Patent are hereby corrected as shown below:

Column 1, line 60, after the word "containing" please insert ---a---. Column 2, line 28, "hertocyclic" should read ---heterocyclic---; line 40, "10<sup>15</sup>" should read ---10<sup>-5</sup>---; line 41, "10<sup>12</sup>" should read ---10<sup>-4</sup>---; line 42, "10" should read ---1---; line 43, "10" should read ---1---; line 52, "2x10<sup>13</sup>" should read ---2x10<sup>-3</sup>---; line 53, "1.5x10<sup>13</sup>" should read ---1.5x10<sup>-3</sup>---; line 55, "10<sup>15</sup>" should read ---10<sup>-5</sup>---; line 56, "2x10<sup>13</sup>" should read ---2x10<sup>-3</sup>---; line 56, after "liter" insert the words ---and preferably from---; line 56, "1x10<sup>14</sup>" should read ---1x10<sup>-4</sup>---; line 57, "1.5x10<sup>13</sup>" should read ---1.5x10<sup>-3</sup>---; line 59, "10<sup>15</sup>" should read ---10<sup>-5</sup>---; line 60, after "moles" please insert ---per liter---; line 60, "4x10<sup>13</sup>" should read ---4x10<sup>-3</sup>---; line 60, "10<sup>14</sup>" should read ---10<sup>-4</sup>---; line 61, "2.5x10<sup>13</sup>" should read ---2.5x10<sup>-3</sup>---; line 61, "10" should read ---per liter---. Column 3, line 19, "photodevelopemnt" should read ---photodevelopment---; line 36, "comprises" should read ---can comprise---. Column 4, line 1, "1x10<sup>16</sup>" should read ---1x10<sup>-6</sup>---; line 2, "10" should read ---1---; line 41, "1" should read ---.1---; line 61, "water-soluble" should read ---water-insoluble---. Column 5, line 6, "from" should read ---form---; line 19, "10<sup>14</sup>" should read ---10<sup>-4</sup>---; line 30, "mercaptotetrazole" should read ---mercaptotetrazole---; line 56, "pyrosolidone" should read ---pyrozolidone---; line 63, "0.48" should be listed directly under the heading ---Background Density---; line 67, "mercaptotetraazole" should read ---mercaptotetrazole---.

UNITED STATES PATENT OFFICE  
CERTIFICATE OF CORRECTION

Patent No. 3,615,511

Dated October 26, 1971

Inventor(s) Roger M. Cole

PAGE - 2

It is certified that error appears in the above-identified patent and that said Letters Patent are hereby corrected as shown below:

Column 6, line 2, "Example 11" should read ---Example 1a---; line 5, "10<sup>14</sup>" should read ---10<sup>-4</sup>---; line 72, "10<sup>14</sup>" should read ---10<sup>-4</sup>---. Column 7, line 13, "1" should be inserted between ---methyl-phenyl---; line 55, "10<sup>14</sup>" should read ---10<sup>-4</sup>---; line 58, "table" should read ---Table---; line 73, "140.0g" should read ---240.0g---. Claim 1, line 5, "10<sup>15</sup>" should read ---10<sup>-5</sup>---; line 6, "2x10<sup>13</sup>" should read ---2x10<sup>-3</sup>---. Claim 6, line 3, "1x10<sup>14</sup>" should read ---1x10<sup>-4</sup>---; line 3, "1.5x10<sup>13</sup>" should read ---1.5x10<sup>-3</sup>---. Claim 7, line 8, "10<sup>15</sup>" should read ---10<sup>-5</sup>---; line 8, "4x10<sup>13</sup>" should read ---4x10<sup>-3</sup>---. Claim 9, line 3, "—" should be inserted between ---2 thiourea---; line 3, "—" should be inserted between ---2 mercaptoimidazole---; Claim 13, line 3, "10<sup>15</sup>" should read ---10<sup>-5</sup>---. Column 3, line 22, "record" should read ---records---.

Page 2 of 2.

Signed and sealed this 9th day of May 1972.

(SEAL)  
Attest:

EDWARD M.FLETCHER, JR.  
Attesting Officer

ROBERT GOTTSCHALK  
Commissioner of Patents